# EUROPEAN PATENT SPECIFICATION

(11) **EP 0 457 589 B1**
(45) Date of publication and mention of the grant of the patent: **10.04.1996**
(21) Application number: 91304405.3
(22) Date of filing: 16.05.1991
(51) Int. Cl.: C10L 1/22

(54) **Fuel compositions with enhanced combustion characteristics**
Kraftstoffzusammensetzungen mit erhöhten Verbrennungseigenschaften
Compositions de combustible à caractéristiques de combustion augmentées

(30) Priority: 17.05.1990 US 524498; 19.11.1990 US 615322
(43) Date of publication of application: 21.11.1991
(73) Proprietor: ETHYL PETROLEUM ADDITIVES, INC., Richmond, Virginia 23219-4304 (US)
(72) Inventor: Cunningham, Lawrence Joseph, Kirkwood, Missouri 63122 (US); Kulinowski, Alexander Michael, St. Louis, Missouri 63125 (US); Henly, Timothy James, St. Louis, Missouri 63119 (US)
(74) Representative: Woods, Geoffrey Corlett

(56) References cited:
- DE-A- 3 233 834
- FR-A- 821 211
- FR-A- 1 349 941
- GB-A- 697 730
- GB-A- 1 547 664
- US-A- 2 031 497
- US-A- 4 073 626
- US-A- 4 328 005
- US-A- 4 448 587
- US-A- 4 561 862

## Description

This invention relates to preservation of the environment. More particularly, this invention relates to fuel compositions and methods that reduce atmospheric pollution normally caused by the operation of engines or combustion apparatus on middle distillate fuels.

The importance and desirability of reducing the release of pollutants into the atmosphere are well recognized. Among the pollutants sought to be reduced are nitrogen oxides ("NOₓ"), carbon monoxide, unburned hydrocarbons, and particulates.

French Patent Specification 821211 describes motor fuels, especially diesel fuels, containing a combustion accelerator, in particular a mixture of dissolved aryl nitrates, to increase the cetane number of the fuel.

This invention involves the discovery, inter alia, that it is possible to reduce the amount of NOₓ or CO or unburned hydrocarbons released into the atmosphere during operation of engines or other combustion apparatus operated on middle distillate fuel by employing as the fuel a middle distillate fuel having a sulfur content of 500 ppm or less and having dissolved there in a combustion improving amount of at least one organic nitrate combustion improver consisting essentially of 2-ethylhexyl nitrate. In fact it has been found possible through use of such fuel compositions to reduce the amount of two and in some cases all three such pollutants (NOₓ, CO and unburned hydrocarbons) emitted by diesel engines. Moreover this important and highly desirable objective has been and thus may be achieved without suffering an undesirable increase in the emission of particulates. This is a unique discovery since the available experimental evidence and mechanistic theories of combustion suggest that if NOₓ is reduced, the amount of particulates will be increased, and vice versa.

Accordingly this invention provides the use of at least one fuel-soluble combustion improver consisting essentially of 2-ethylhexyl nitrate, incorporated in a hydrocarbonaceous middle distillate fuel having a sulfur content of less than 500 ppm prior to combustion in a proportion of 1000 to 5000 parts by weight per million parts of fuel for reducing emissions of at least two of NOₓ, CO and unburned hydrocarbons during combustion of said fuel, having the distillation profile disclosed in claim 1 and page 6, in a diesel engine in the presence of air.

The hydrocarbonaceous middle distillate fuel preferably has a sulfur content of 100 ppm or less and most preferably no more than 60 ppm. By the term "hydrocarbonaceous" as used in the ensuing description and appended claims is meant the middle distillate fuel is composed principally or entirely of fuels derived from petroleum by any of the usual processing operations. The finished fuels may contain, in addition, minor amounts of non-hydrocarbonaceous fuels or blending components such as alcohols, dialkyl ethers, or like materials, and/or minor amounts of suitably desulfurized auxiliary liquid fuels of appropriate boiling ranges (i.e. between about 160 and about 370°C) derived from tar sands, shale oil or coal. When using blends composed of such desulfurized auxiliary liquid fuels and hydrocarbonaceous middle distillate fuels, the sulfur content of the total blend must be kept below 500 ppm.

This invention thus provides improvements in the operation of motor vehicles and aircraft which operate on middle distillate fuels. These improvements involve fuelling the vehicle or aircraft with a hydrocarbonaceous middle distillate fuel having a sulfur content of less than 500 ppm (preferably 100 ppm or less and most preferably no more than 60 ppm) and containing the aforesaid organic nitrate combustion improver dissolved therein.

In accordance with a particularly preferred embodiment of this invention, there is provided the use of a hydrocarbonaceous middle distillate fuel having a sulfur content of not more than 500 ppm (preferably 100 ppm or less and most preferably no more than 60 ppm) and a 10% boiling point (ASTM D-86) in the range of about 154° to about 230°C, said fuel containing a minor combustion improving amount of at least one fuel-soluble organic nitrate combustion improver consisting essentially of 2-ethylhexyl nitrate. Such fuel compositions tend on combustion to emit especially low levels of NOₓ. Without desiring to be bound by theoretical considerations, one explanation for such highly desirable performance is that fuels with higher 10% boiling points cause a delay in the progression of combustion and consequent higher peak temperatures which increase the amount of NOₓ formation.

Pursuant to another particularly preferred embodiment of this invention there is provided the use of a hydrocarbonaceous middle distillate fuel having a sulfur content of not more than 500 ppm (preferably 100 ppm or less and most preferably no more than 60 ppm) and a 90% boiling point (ASTM D-86) in the range of about 260° to about 320°C, said fuel containing a minor combustion improving amount of at least one fuel-soluble organic nitrate combustion improver consisting essentially of 2-ethylhexyl nitrate. Such fuel compositions tend on combustion to emit especially low levels of particulates.

These and other embodiments are set forth in the ensuing description and appended claims.

In the accompanying drawings:
Fig. 1 is a least-squares plot of NOₓ emissions versus 10% boiling temperatures of fuels having a nominal cetane number of approximately 50; and
Fig. 2 is a least-squares plot of particulate emissions versus 90% boiling temperatures of fuels having a nominal cetane number of approximately 50.

The hydrocarbonaceous fuels utilized in the practice of this invention are comprised in general of mixtures of hydrocarbons which fall within the distillation range of about 160 to about 370°C. Such fuels are frequently referred to as "middle distillate fuels" since they comprise the fractions which distill after gasoline. Such fuels include diesel fuels, burner fuels, kerosenes, gas oils, jet fuels, and gas turbine engine fuels.

The used middle distillate fuels are those characterized by having the following distillation profile:

| | °F | °C |
|---|---|---|
| IBP | 250 - 500 | 121 - 260 |
| 10% | 310 - 550 | 154 - 288 |
| 50% | 350 - 600 | 177 - 316 |
| 90% | 400 - 700 | 204 - 371 |
| EP | 450 - 750 | 232 - 399 |

Diesel fuels having a clear cetane number (i.e., a cetane number when devoid of any cetane improver such as an organic nitrate) in the range of 30 to 60 are preferred. Particularly preferred are those in which the clear cetane number is in the range of 40 to 50.

The organic nitrate combustion improvers (also frequently known as ignition improvers) comprise nitrate esters of substituted or unsubstituted aliphatic or cycloaliphatic alcohols which may be monohydric or polyhydric. Preferred organic nitrates are substituted or unsubstituted alkyl or cycloalkyl nitrates having up to about 10 carbon atoms, preferably from 2 to 10 carbon atoms. The alkyl group may be either linear or branched (or a mixture of linear and branched alkyl groups). Specific examples of nitrate compounds suitable for use as nitrate combustion improvery include, but are not limited to, the following: methyl nitrate, ethyl nitrate, n-propyl nitrate, isopropyl nitrate, allyl nitrate, n-butyl nitrate, isobutyl nitrate, sec-butyl nitrate, tert-butyl nitrate, n-amyl nitrate, isoamyl nitrate, 2-amyl nitrate, 3-amyl nitrate, tert-amyl nitrate, n-hexyl nitrate, n-heptyl nitrate, sec-heptyl nitrate, n-octyl nitrate, 2-ethylhexyl nitrate, sec-octyl nitrate, n-nonyl nitrate, n-decyl nitrate, cyclopentylnitrate, cyclohexyl nitrate, methylcyclohexyl nitrate, isopropylcyclohexyl nitrate, and the like. Also suitable are the nitrate esters of alkoxy substituted aliphatic alcohols such as 2-ethoxyethyl nitrate, 2-(2-ethoxyethoxy)ethyl nitrate, 1-methoxypropyl-2-nitrate, and 4-ethoxybutyl nitrate, as well as diol nitrates such as 1,6-hexamethylene dinitrate, and the like. Preferred are the alkyl nitrates having from 5 to 10 carbon atoms, most especially mixtures of primary amyl nitrates, mixtures of primary hexyl nitrates, and octyl nitrates such as 2-ethylhexyl nitrate.

As is well known, nitrate esters are usually prepared by the mixed acid nitration of the appropriate alcohol or diol. Mixtures of nitric and sulfuric acids are generally used for this purpose. Another way of making nitrate esters involves reacting an alkyl or cycloalkyl halide with silver nitrate.

The concentration of nitrate ester in the fuel can be varied within relatively wide limits such that the amount employed is at least sufficient to cause a reduction in emissions. This amount falls within the range of 1,000 to 5,000 parts by weight per million parts of fuel.

Other additives may be included within the fuel compositions of this invention provided they do not adversely affect the exhaust emission reductions achievable by the practice of this invention. Thus use may be made of such components as organic peroxides and hydroperoxides, corrosion inhibitors, antioxidants, antirust agents, detergents and dispersants, friction reducing agents, demulsifiers, dyes, inert diluents, and like materials.

The advantages achievable by the practice of this invention were demonstrated in a sequential series of engine tests in which a Detroit Diesel 11.1 liter Series 60 engine mounted to an engine dynamometer was used. The system was operated on the "EPA Engine Dynamometer Schedule for Heavy-Duty Diesel Engines" set forth at pages 810-819 of Volume 40, Part 86, Appendix I, of the Code of Federal Regulations (7-1-86). In these tests, the first of five consecutive tests involved operation of the engine on a conventional DF-2 diesel fuel having a nominal sulfur content in the range of 2000 to 4000 ppm. This test served as one of two baselines. In the next operation the engine was run using a low-sulfur diesel fuel having the following characteristics:

| | |
|---|---|
| Sulfur, ppm | 50 |
| Gravity, API @ 60°F (15.5°C) | 34.7 |
| Pour Point, °F (°C) | - 5 (-20) |
| Cloud Point, °F (°C) | 8 (-13) |
| Copper Strip | 1 |
| Distillation, °F (°C) | |
| IBP | 332 (167) |
| 10% | 430 (221) |
| 50% | 532 (278) |
| 90% | 632 (333) |
| EP | 634 (334) |
| Cetane Number | 44.3 |
| Viscosity @ 40°C, cS | 2.96 |

In the third and fourth tests -- which represented the practice of this invention -- this same low-sulfur fuel was used except that it had blended therein a diesel ignition improver composed of 2-ethylhexyl nitrate. In the third test the concentration was 2000 ppm of the organic nitrate. In the fourth test, the fuel contained 5000 ppm of the organic nitrate. The fifth and final test involved another baseline run using the initial conventional DF-2 diesel fuel. In all instances the quantities of NOₓ, unburned hydrocarbons ("HC"), carbon monoxide ("CO") and particulates emitted by the engine were measured and integrated. The results of these tests are summarized in the following table. The values shown therein for NOₓ, HC, CO, and Particulates, are presented in terms of grams per brake horsepower per hour (i.e. grams per 745 watts per hour). Thus the lower the value, the lower the rate and amount of emissions.

| Test No. | NOx | HC | CO | Particulates |
|---|---|---|---|---|
| 1 | 4.641 | 0.086 | 1.414 | 0.227 |
| 2 | 4.345 | 0.068 | 1.490 | 0.165 |
| 3 | 4.173 | 0.051 | 1.312 | 0.164 |
| 4 | 4.208 | 0.073 | 1 324 | 0.165 |
| 5 | 4.623 | 0.078 | 1.525 | 0.223 |

In particularly preferred embodiments of this invention, use of fuels having certain boiling characteristics as well as low sulfur levels, results in still further reductions in either NOₓ or particulate emissions. Thus by use of fuels meeting the low sulfur parameters set forth hereinabove and additionally having a 10% boiling point (ASTM D-86) in the range of 154-230°C, the emissions of NOₓ can be reduced to extremely low levels. Likewise, by use of fuels meeting the low sulfur parameters set forth hereinabove and additionally having a 90% boiling point (ASTM D-86) in the range of 260-320°C, particulate emissions tend to be reduced to especially low levels. To illustrate, a Detroit Diesel Corporation Series 60 Engine in the 11.1 liter configuration and nominally rated at 320 hp at 1800 rpm was used in a series of emission tests. The engine was installed in a heavy-duty transient emission cell equipped with a constant volume sampler (CVS) system. A dilution tunnel permitted measurements of HC, CO, NOₓ and particulates according to the EPA Transient Emissions Cycle Procedure.

For each individual test case, the engine was started and warmed up. It was then run for 20 minutes at rated speed and load. Rated power was validated. In addition, a power test was conducted, mapping engine torque vs. speed. These parameters are required as part of the EPA Transient Cycle Procedure. Once this information was obtained, two 20-minute EPA Transient Cycles were run and engine controls were adjusted to meet statistical operating limits prescribed for the tests. The engine was shut down and allowed to soak for 20 minutes. At the end of the soak period, the Hot Start EPA Transient Cycle was run to measure NOₓ, CO and particulate emissions. A second emissions evaluation was conducted after another two-minute soak. Results for the two Hot Transient Cycles were averaged into a final reported value. Whenever a fuel was changed, new fuel was introduced into the fueling system, new fuel filters were installed, and fuel lines were flushed.

Each fuel (A through D) was evaluated by the same Hot Start EPA Transient Emissions Cycle Procedure. Fuels A, B, and C contained 2-ethylhexyl nitrate in an amount sufficient to raise the cetane number of the respective fuels to a nominal value of 50. Fuel D which had a natural cetane number of 49.8 was used unadditized.

Physical and chemical characterization data for unadditized fuels A through D are shown in the following table:

**TABLE**

| Fuel Property | A | B | C | D |
|---|---|---|---|---|
| Hydrocarbon Composition, vol % | | | | |
| Aromatics | 36.5 | 28.5 | 37.6 | 39.4 |
| Olefins | 1.2 | 1.1 | 2.2 | 2.9 |
| Saturates | 62.3 | 70.4 | 60.2 | 57.7 |
| | | | | |
| Carbon, wt% | 86.35 | 86.49 | 86.12 | 87.32 |
| Hydrogen, wt% | 13.15 | 13.25 | 12.89 | 13.35 |
| Nitrogen, ppm | 5.3 | 285 | 356 | 152 |
| Sulfur, ppm | <1 | 225 | 219 | 476 |
| | | | | |
| Aniline pt., deg. C | 70.1 | 60.0 | 65.4 | 69.4 |
| Diene content, wt% | <0.1 | 0.2 | <0.1 | <0.1 |
| | | | | |
| Viscosity, cSt | | | | |
| @ 40 deg. C | 2.99 | 2.20 | 3.10 | 3.53 |
| @ 100 deg. C | 1.22 | 0.97 | 1.23 | 1.34 |
| | | | | |
| Heat of combustion BTU/lb(kJ/g) | 19,593 | 19,840 | 19,543 | 19,672 |
| | (45.6) | (46.1) | (45.5) | (45.8) |
| Boiling range, deg. C | | | | |
| IBP | 170 | 172 | 202 | 218 |
| 10% | 217 | 211 | 234 | 252 |
| 20% | 233 | 222 | 246 | 262 |
| 30% | 249 | 230 | 257 | 271 |
| 40% | 262 | 237 | 267 | 278 |
| 50% | 274 | 244 | 276 | 284 |
| 60% | 288 | 253 | 286 | 291 |
| 70% | 300 | 263 | 294 | 298 |
| 80% | 314 | 276 | 306 | 306 |
| 90% | 331 | 297 | 322 | 317 |
| 95% | 344 | 319 | 338 | 329 |
| FBP | 352 | 334 | 353 | 341 |
| Recovery, % | 98.7 | 98.9 | 98.6 | 98.9 |
| | | | | |
| Gravity, deg. API | 34.9 | 36.1 | 34.6 | 34.5 |
| Specific gravity | 0.850 | 0.844 | 0.852 | 0.852 |
| | | | | |
| Calculated cetane index | 48.1 | 44.0 | 48.9 | 51.7 |
| Cetane index | 48.5 | 43.8 | 48.3 | 49.7 |
| Cetane number | 45.3 | 39.6 | 47.7 | 49.8 |

In the above table, the following test methods were used:
Hydrocarbon composition - ASTM D-1319
Carbon - Carlo-Erba 1106
Hydrogen - Carlo-Erba 1106
Nitrogen - ASTM D-4629
Sulfur - ASTM D-3120
Aniline pt. - ASTM D-611
Diene content - UOP 326
Viscosity - ASTM D-445
Heat of combustion - ASTM D-2382
Boiling range - ASTM D-86
Gravity - ASTM D-287
Calculated cetane index - ASTM D-4737
Cetane index - ASTM D-976
Cetane number - ASTM D 613

Fig. 1 presents graphically the results of NOₓ emissions in relation to the 10% boiling temperatures of the four fuels. It can be seen that the fuels in which the 10% boiling temperature was below 230°C had the lowest NOₓ emissions.

The results of the particulate determinations are graphically depicted in Fig. 2. In this case, the results are shown as a function of 90% boiling temperatures of the base fuels. A trend toward lower particulate emissions with fuels having 90% boiling points within the range of 260-320°C was noted.

Methods for reducing the sulfur content of hydrocarbonaceous middle distillate fuels or their precursors are reported in the literature and are otherwise available to those skilled in the art. Among such processes are solvent extraction using such agents as sulfur dioxide or furfural, sulfuric acid treatment, and hydrodesulfurization processes. Of these, hydrodesulfurization is generally preferred, and includes a number of specific methods and operating conditions as applied to various feedstocks. For example, hydrotreating or hydroprocessing of naphthas or gas oils is generally conducted under mild or moderate severity conditions. On the other hand, sulfur removal by hydrocracking as applied to distillate stocks is usually conducted under more severe operating conditions. Vacuum distillation of bottoms from atmospheric distillations is still another method for controlling or reducing sulfur content of hydrocarbon stocks used in the production of hydrocarbonaceous middle distillate fuels. Further information concerning such processes appears in Kirk-Othmer, Encyclopedia of Chemical Technology, Second Edition, Interscience Publishers, Volume 11, pages 432-445 (copyright 1966) and references cited therein; Idem., Volume 15, pages 1-77 and references cited therein; and Kirk-Othmer, Encyclopedia of Chemical Technology, Volume 17, Third Edition, Wiley-Interscience, pages 183-256 (copyright 1982) and references cited therein. All of such publications and cited references are incorporated herein by reference in respect of processes or methods for control of reduction of sulfur content in hydrocarbonaceous middle disillate fuels or their precursor stocks.

Another method which can be used involves treatment of the hydrocarbonaceous middle distillate fuel with a metallic desulfurization agent such as metallic sodium, or mixtures of sodium and calcium metals.

Other similar embodiments of this invention will readily occur to those skilled in the art from a consideration of the foregoing disclosure.

## Claims

1. The use of a fuel-soluble combustion improver consisting essentially of 2-ethylhexyl nitrate incorporated in a hydrocarbonaceous middle distillate fuel, said fuel having the following distillation profile:
| | °C |
|---|---|
| IBP | 121-260 |
| 10% | 154-288 |
| 50% | 177-316 |
| 90% | 204-371 |
| EP | 232-399 |
and having a sulfur content of less than 500 ppm, prior to combustion in a proportion of 1000 to 5000 parts by weight per million parts of fuel for reducing emissions of at least two of NOₓ, CO and unburned hydrocarbons during combustion of said fuel in a diesel engine in the presence of air.

2. The use of claim 1, wherein the base fuel has a sulfur content of 100 ppm or less and a clear cetane number in the range of 30 to 60.

3. The use of claim 1, wherein the base fuel has a sulfur content of no more than 60 ppm.

4. The use of claim 3, wherein the base fuel has a clear cetane number in the range of 50 to 60.

5. The use of claim 3, wherein the base fuel has a clear cetane number in the range of 40 to 50.

6. The use of any one of the preceding claims, wherein emissions of NOₓ, CO and unburned hydrocarbons are reduced.

7. The use of any one of the preceding claims, wherein the base fuel has a 10% boiling point (ASTM D-86) in the range of 154-230°C.

8. The use of any one of the preceding claims, wherein the base fuel has a 90% boiling point (ASTM D-86) in the range of 260-320°C.

## Patentansprüche

1. Verwendung eines in Treibstoff löslichen Mittels zur Verbesserung der Verbrennung, das im wesentlichen aus in einen Mitteldestillattreibstoff aus Kohlenwasserstoffen eingearbeitetem 2-Ethylhexylnitrat besteht, wobei der Treibstoff das folgende Destillationsprofil:
| | °C |
|---|---|
| IBP | 121-260 |
| 10% | 154-288 |
| 50% | 177-316 |
| 90% | 204-371 |
| EP | 232-399 |
und einen Schwefelgehalt von weniger als 500 ppm, vor der Verbrennung in einer Menge von 1000 bis 5000 Gewichtsanteilen auf eine Million Teile Treibstoff aufweist, um die Emissionen von mindestens zwei aus der Reihe NOₓ, CO und nichtverbrannten Kohlenwasserstoffen während der Verbrennung des Treibstoffs in einem Dieselmotor in Anwesenheit von Luft zu verringern.

2. Verwendung gemäß Anspruch 1, bei der der Grundtreibstoff einen Schwefelgehalt von 100 ppm oder weniger und eine reine Cetanzahl im Bereich von 30 bis 60 aufweist.

3. Verwendung gemäß Anspruch 1, bei der der Grundtreibstoff einen Schwefelgehalt unterhalb von 60 ppm aufweist.

4. Verwendung gemäß Anspruch 3, bei der der Grundtreibstoff eine reine Cetanzahl im Bereich von 50 bis 60 hat.

5. Verwendung gemäß Anspruch 3, bei der der Grundtreibstoff eine reine Cetanzahl im Bereich von 40 bis 50 hat.

6. Verwendung gemäß einem der vorstehenden Ansprüche, bei der die Emissionen an NOₓ, CO und nichtverbrannten Kohlenwasserstoffen reduziert sind.

7. Verwendung gemäß einem der vorstehenden Ansprüche, bei der der Grundtreibstoff einen 10 %igen Siedepunkt (ASTM D-86) im Bereich von 154 - 230°C hat.

8. Verwendung gemäß einem der vorstehenden Ansprüche, bei der der Grundtreibstoff einen 90 %igen Siedepunkt (ASTM D-86) im Bereich von 260 - 320 °C hat.

## Revendications

1. Utilisation d'un agent améliorant la combustion, soluble dans les carburants, consistant essentiellement en nitrate de 2-éthylhexyle incorporé à un carburant consistant en un distillat moyen hydrocarboné, ledit carburant ayant le profil de distillation suivant :
| | °C |
|---|---|
| IBP | 121-260 |
| 10% | 154-288 |
| 50% | 177-316 |
| 90% | 204-371 |
| EP | 232-399 |
et ayant une teneur en soufre inférieure à 500 ppm, avant combustion, en une proportion de 1000 à 5000 parties en poids par million de parties de carburant pour réduire les émissions d'au moins deux des composés consistant en NOₓ, CO et hydrocarbures imbrûlés au cours de la combustion dudit carburant dans un moteur diesel en présence d'air.

2. Utilisation suivant la revendication 1, dans laquelle le carburant de base a une teneur en soufre égale ou inférieure à 100 ppm et un indice de cétane clair compris dans l'intervalle de 30 à 60.

3. Utilisation suivant la revendication 1, dans laquelle le carburant de base a une teneur en soufre non supérieure à 60 ppm.

4. Utilisation suivant la revendication 3, dans laquelle le carburant de base a un indice de cétane clair compris dans l'intervalle de 50 à 60.

5. Utilisation suivant la revendication 3, dans laquelle le carburant de base a un indice de cétane clair compris dans l'intervalle de 40 à 50.

6. Utilisation suivant l'une quelconque des revendications précédentes, dans laquelle les émissions de NOₓ, de CO et d'hydrocarbures imbrûlés sont réduites.

7. Utilisation suivant l'une quelconque des revendications précédentes, dans laquelle le carburant de base a un point d'ébullition à 10 % (ASTM D-86) compris dans l'intervalle de 154 à 230°C.

8. Utilisation suivant l'une quelconque des revendications précédentes, dans laquelle le carburant de base a un point d'ébullition à 90 % (ASTM D-86) compris dans l'intervalle de 260 à 320°C.
